

1,159,713.

L. G. ROWAND.  
SEPARATION OF MINERALS BY FLOTATION.  
APPLICATION FILED AUG. 1, 1914.

Patented Nov. 9, 1915.



WITNESSES

WITNESSED  
M. A. Bill  
Kernett, ~~John~~ <sup>John</sup> A. Bill

*INVENTOR:*

INVENTOR:  
Lewis G. Howard,  
BY  
Fannie, Davis & Goldsborough,  
ATTORNEYS.

# UNITED STATES PATENT OFFICE.

LEWIS G. ROWAND, OF BROOKLYN, NEW YORK, ASSIGNOR TO NEW JERSEY ZINC COMPANY, OF NEW YORK, N. Y., A CORPORATION OF NEW JERSEY.

## SEPARATION OF MINERALS BY FLOTATION.

1,159,713.

Specification of Letters Patent.

Patented Nov. 9, 1915.

Application filed August 1, 1914. Serial No. 854,529.

To all whom it may concern:

Be it known that I, LEWIS G. ROWAND, a citizen of the United States, residing in the borough of Brooklyn, county of Kings, State of New York, have invented certain new and useful Improvements in the Separation of Minerals by Flotation; and I do hereby declare the following to be a full, clear, and exact description of the invention, such as will enable others skilled in the art to which it appertains to make and use the same.

The present invention relates to the separation of metalliferous values from ores, slimes, and the like, wherein the minerals to be separated are associated with gangue, or other minerals not susceptible of selective flotation by the oil, emulsion, or the like, employed for that purpose.

The characteristic feature of the invention consists in feeding the material to be treated upon a traveling belt or apron or other moving surface which receives a layer of the separating oil or emulsion by contact with a suitable source of supply, and which feeds the material, after it has been deposited upon the layer of oil or emulsion carried by the belt, into a flotation tank, in such manner that it will enter the water in the tank at the surface thereof; whereupon the particles susceptible of flotation will be floated off into a collecting trough or launder, and the particles not capable of flotation will drop through the water contained in the tank and will be collected separately as tailings. In passing down the incline, the metalliferous particles to be separated will take on a surface coating of the oil, emulsion, or the like, whereas the particles which have no tendency to become coated remain unaffected; consequently, when the mass of material is fed, at a suitably moderate rate upon the surface of the water, the coated particles, representing corresponding metalliferous values, will be buoyed up and floated off into the collecting launder for heads, whereas the uncoated particles will fall by gravity to the bottom of the flotation tank.

In the accompanying drawing,—Figure 1 represents a cross-sectional view, partly in elevation, of apparatus adapted for the practice of the invention; Fig. 2 represents a similar fragmentary view on a larger scale and illustrates generally the mode of operation of the invention.

Similar letters of reference indicate similar parts in both views.

Referring to the drawing A, indicates a flotation tank having an inclined bottom and provided with a hand valve *a* for the discharge of the tailings. The tank A is supplied with the flotation liquid (for instance, water), through a pipe provided with a cut-off valve *b*, and the tank has a collecting or conveying trough or launder *c*, which receives the heads as they are floated over the verge *d*. By means of the hand valve *b* the water or other liquid may be supplied in such volume as to maintain the necessary depth of overflow at the verge *d*, so that the floating particles will clear the verge in passing over into the collecting launder.

The moving surface upon which the ore to be separated is received is preferably, as shown, a belt or apron *e*, which passes over the rollers *f*, *g*, either one of which may be provided with power to rotate it and thus cause the belt or apron *e* to move at an appropriate rate, in the direction indicated by the arrows.

*h* indicates an idler roll, which may have the two-fold function of a belt tightener and a means for lifting the lower strand of the belt or apron so that it shall clear the wall *i* of the flotation tank.

*B* indicates a suitable chute for supplying the material to the upper surface of the top strand of the belt or apron.

Adjacent to the flotation tank is located a receptacle *D* for the oil, emulsion of oil and acid, or like liquid having a selective floatation effect upon the metalliferous particles which it is designed to recover as heads, in the practice of the invention. This receptacle *D* may conveniently be built in one with the flotation tank, as shown, and is preferably provided with an inclined bottom and a hand discharge valve *k*. It may be supplied in any suitable manner, as, for instance, by the supply pipe *m*.

I do not limit myself to any particular oil, emulsion, or other liquid for the filling of the receptacle *D*, inasmuch as the particular liquid selected will depend upon the character of the ore treated and particularly the character of its metalliferous values.

Whatever the liquid selected for the filling of the receptacle *D*, the arrangement is such that the traveling belt or apron will be

carried down into contact with said liquid and will receive a surface coating or layer thereof, as indicated at *n* in Fig. 2. The ore, (suitably crushed or otherwise reduced to a sufficiently fine state of sub-division, familiar to those skilled in the art,) or the slimes, as the case may be, will be fed upon the upper surface of the belt or apron *e* in such manner as to be distributed thereon to the best advantage and in a thin layer.

The general mode of operation is indicated in Fig. 2, which illustrates the taking up by the metalliferous values, by surface tension, of the oil, emulsion, or the like, as an enveloping coating, whereas the particles shown as uncoated represent constituents of the gangue.

The material is fed by the belt, at a sufficiently moderate rate of speed to permit the water to exert its best buoyancy effect upon the coated metalliferous particles, whereupon they are buoyed up for the most part at the surface of the water and are floated off into the launder.

Other coated particles which may be carried downward to a greater or less depth by entanglement with the gangue likewise tend to reach the surface of the water and to join the heads in their overflow from the flotation tank.

What I claim is:

1. The method of separating sulfid constituents from ores in which they are contained, which comprises feeding the solid particles of the ore in a finely divided condition upon a moving layer of an oleaginous liquid having a selective action for the sulfids of a character to effect flotation, progressively feeding said layer with its charge of ore into a flotation liquid at the surface thereof, and floating off and recovering the floating sulfids; substantially as described.

2. The method of separating metal-carrying constituents from ores in which they are contained, which comprises feeding the ore in a finely divided condition upon a traveling apron having a surface coating of an

oleaginous substance having a selective action for the metal-carrying constituents of a character to effect their flotation, and progressively feeding said apron with its charge of ore into an aqueous flotation liquid at the surface thereof; substantially as described.

3. Apparatus for effecting, by flotation, the separation of metal-carrying constituents from ores in which they are contained, which comprises a flotation tank, a traveling apron whose delivery end discharges into said tank at the overflow level thereof, means for supplying to the surface of the apron a layer of liquid having a selective action for the metal-carrying constituents of a character to effect their flotation, means for feeding the ore to be separated, in a finely divided condition upon the layer of selective liquid, and means for effecting the overflow of the flotation tank and the progressive recovery of the floated constituents; substantially as described.

4. Apparatus for effecting, by flotation, the separation of metal-carrying constituents upon ores in which they are contained, which comprises a flotation tank, a traveling apron whose delivery end discharges into said tank at the overflow level thereof, means for supplying to the surface of the apron a layer of liquid having a selective action for the metal-carrying constituents of a character to effect their flotation, said means consisting of a receptacle for said selective liquid into which the traveling belt dips, means for feeding the ore to be separated in a finely divided condition upon the layer of selective liquid, said means consisting of a feeding device for dropping the finely divided ore upon the layer of selective liquid; substantially as described.

In testimony whereof I affix my signature in presence of two witnesses.

LEWIS G. ROWAND.

Witnesses:

IRA S. HELLER,  
J. T. HAMINGAN.

Copies of this patent may be obtained for five cents each, by addressing the "Commissioner of Patents, Washington, D. C."